

May 12, 1959

G. R. SCHAEER ET AL

2,886,499

PROTECTIVE METAL COATINGS FOR MOLYBDENUM

Filed Jan. 7, 1957



FIG. 3

INVENTORS  
JOHN G. BEACH  
GLEN R. SCHAEER

BY

H. W. Zosche  
ATTORNEYS

# United States Patent Office

2,886,499

Patented May 12, 1959

1  
2,886,499

PROTECTIVE METAL COATINGS FOR

MOLYBDENUM

Glenn R. Schaer and John G. Beach, Columbus, Ohio, assignors, by mesne assignments, to the United States of America as represented by the Secretary of the Navy

Application January 7, 1957, Serial No. 632,951

3 Claims. (Cl. 204—41)

The present invention relates to metal coatings for molybdenum and more particularly to electroplated coatings that will act as a barrier to the diffusion of molybdenum through the coatings.

It is well known that molybdenum, as well as other refractory metals, is readily oxidized when exposed to an oxygen-bearing atmosphere at elevated temperatures. As molybdenum and molybdenum base alloys have high strength at elevated temperatures, it is desirable to provide satisfactory oxidation resistance for these materials so that their use can be expanded. It has been the customary practice to electroplate molybdenum with various other metals, such as nickel and chromium, to prevent the oxidation of the molybdenum. A protective electroplated metal at a high temperature must not only resist oxidation from the environment in which the coating will be placed but must also prevent deterioration of the basis metal caused by the environment. The oxidation resistance of most commercially usable electrodeposited metals is dependent upon the formation of an adherent and impervious oxide coating. In addition to oxidation resistance, the electroplate and its scale must withstand impact and abrasion, stress corrosion and creep. If the electroplate diffuses rapidly with the basis metal, the coating life is shortened. Discontinuities in the coating reduce its ability to protect the basis metal, and therefore the density and structure of electrodeposits are important.

Although nickel resists oxidation in air better than chromium under conditions of cyclic heating, chromium can be deposited on molybdenum with a better adherence than is possible by plating nickel and several other electrodeposits directly on molybdenum. However, at high temperatures, the molybdenum diffuses through the chromium plating, causing shrinkage of the molybdenum, and, furthermore, molybdenum and/or oxygen diffusing through the plating and reacting with each other at high temperatures forms a liquid or gas that corrodes chromium, nickel, and other metals faster than does air.

The present invention provides an improved method for coating molybdenum and molybdenum base alloys by first depositing chromium on molybdenum and then applying a deposit of gold over the layer of chromium. A protective layer of chromium can then be deposited over the layer of gold. At elevated temperatures, gold only slightly retards the diffusion of chromium through the gold and into the molybdenum, but diffusion of the molybdenum through the resulting gold-chromium diffusion alloy is effectively retarded.

It is therefore a general object of the present invention to provide an improved coating for molybdenum whereby the rapid oxidation of the molybdenum at high temperatures is effectively retarded.

Other objects and many of the attendant advantages of this invention will be readily appreciated as the same becomes better understood by reference to the following detailed description when considered in connection with the accompanying drawing wherein:

2

Figure 1 is a partial sectional view showing chromium and gold plating on a molybdenum specimen;

Figure 2 is a sectional view illustrating a microscopic view of an electroplated molybdenum specimen, after heating, and

Figure 3 is a diagram showing the growth of a molybdenum-chromium diffusion zone with time at various temperatures.

As shown in Figure 1 of the drawing, the present invention contemplates first applying a strike coating (approximately 0.0005 inch) of chromium 11 on the molybdenum 12 in order that the subsequent gold plate 13 will be deposited adherently. The base metal is cleansed and prepared for plating in any conventional manner and then plated with chromium. By way of example, the molybdenum objects to be plated can be heat treated in hydrogen for 2 hours at 980° C., cooled, immersed in nitric acid solution (3HNO<sub>3</sub>:1H<sub>2</sub>O) for 10 seconds, rinsed, electro-etched 2 minutes at 350 amp./sq. ft. (85° F.) in a solution containing 100 g./l. chromic acid and 10 g./l. sodium dichromate, rinsed, immersed in 15 percent, by weight, of hydrochloric acid solution, rinsed, and plated with chromium at 185° F. with a current density of 900 amp./sq. ft. for 1 to 5 minutes.

After the molybdenum specimens have been given a strike coating of chromium, a .0015 inch gold layer is deposited. By way of example, the specimens are immersed in 15 percent, by weight, hydrochloric acid solution for 5 seconds at 85° F., rinsed, and then plated in a gold plating bath, having the following formulation and operating conditions:

*Formulation*  
40 g./l. potassium gold cyanide

29 g./l. potassium cyanide  
40 g./l. potassium tartrate  
3 g./l. potassium hydroxide  
10 g./l. potassium carbonate

12.0 pH  
*Operating conditions*

Cathode current density ----- 5 or 10 amp./sq. ft.

Anodes ----- 24K gold.

Bath temperature ----- 130° F.

Agitation ----- None.

Plating rate ----- 0.0015 inch/hour  
at 10 amp./sq. ft.

After plating with gold, a heavier coating of chromium 14 (.003—.005 inch) is then deposited over the layer of gold. By way of example, the heavier layer of chromium 14 can be plated by using the following formulation and operating conditions:

*Formulation*

250 g./l. chromic acid  
2.5 g./l. sulfuric acid

*Operating conditions*

Cathode current density ----- 750 amp./sq. ft.

Anodes ----- Chemical lead sheet.

Bath temperature ----- 185° F.

Plating time ----- Approximately 3—5 hours.

Referring now to Figure 2 of the drawing, there is shown a view, as might be observed under a microscope, of an electroplated molybdenum specimen that has been heated, wherein the heating caused a progressive growth of a molybdenum-chromium diffusion zone 15 under the gold. Microscopic thickness measurements of sections heated for 25, 57, and 100 hours showed that the alloy zone grows at nearly the same rate as the diffusion alloy grows between molybdenum and chromium, as shown in

Figure 3 of the drawing. For example, one molybdenum specimen that was first given a .0005 inch thick chromium strike, followed by a .0015 inch plating of gold, and then .004 inch of chromium, was heated for 100 hours at 980° C. in argon atmosphere, and the diffusion zone in the gold and chromium plated molybdenum section, shown in Figure 2, was about .00075 inch thick, whereas the diffusion zone after 100 hours for chromium plated molybdenum (without gold) would be about .0009 inch thick, as shown in Figure 3 of the drawing.

The diffusion zone 15, consisting of two layer-like phases between the gold and the molybdenum, is a white alloy with a hardness of 470 Knoop. It contained little, if any, gold because the intermetallic compounds of gold and molybdenum are very much harder. The hardness of the yellow-gold layer 16 above the chromium-molybdenum zone 15 indicates that, upon heating, a significant proportion of chromium is alloyed with the gold. The hardness of the gold-chromium alloy 16 is 199 Knoop, whereas annealed gold has a hardness of less than 40 Knoop. The hardness of the chromium 14 above the gold alloy is 180 Knoop, and, because this value corresponds to the hardness of annealed, electrolytic chromium, it is evident that no molybdenum or gold diffuses into the outer layer of chromium. Thus it is evident that the molybdenum base metal 12 is adequately protected from oxidation at high temperatures by the layers of chromium and gold.

During microscopic examination of electroplated molybdenum specimens, several gaps in the gold alloy layer were observed. Whenever the gaps appeared, the white diffusion alloy below the gold alloy was very narrow. These observations show that the gap retarded the diffusion of chromium with molybdenum. Because the growth of the white diffusion zone depended upon the diffusion of chromium through gold, the white diffusion zone evidently contained little, if any, gold.

After molybdenum or molybdenum base alloys are coated with a diffusion barrier as described above, it may be desirable to apply an additional oxidation resistant metal over the outer coating of chromium 14. In particular, under conditions of cyclic heating, the electroplating of a nickel coating over the chromium coating 14 is highly desirable. Although chromium is ordinarily considered

more resistant than nickel to oxidation in air, nickel is actually more resistant under conditions of cyclic heating, the reason for this apparently being due to the fact that the nickel forms a tightly adherent nickel oxide surface coating. On the other hand, the chromium oxide scale formed on the chromium surface is not as adherent as the nickel oxide scale formed on the nickel surface.

Obviously many modifications and variations of the present invention are possible in the light of the above teachings. It should therefore be understood that it is intended that all matter contained in the above description and drawing shall be interpreted as illustrative and not in a limiting sense.

What is claimed is:

15. The method of protecting molybdenum articles from oxidation at high temperatures comprising, first electroplating said articles with a strike coating of chromium about .0005 inch thick, next electroplating a layer of gold about .0015 inch thick on said strike coating of chromium, and finally electroplating a layer of chromium from .003 to .005 inch thick on said layer of gold.
20. The method of protecting articles of molybdenum and molybdenum base alloys from oxidation at high temperatures comprising, electroplating a strike coating of chromium about .0005 inch thick on said articles, next electroplating a coating of gold about .0015 inch thick thereon, then electroplating a substantially thicker coating of chromium from .003 to .005 inch thick on said gold coating, and then electroplating thereover an outside coating of a metal resistant to oxidation under cyclic heating.
25. The method of protecting articles of molybdenum and molybdenum base alloys as set forth in claim 2 wherein said outside coating of metal is nickel.

35. References Cited in the file of this patent

UNITED STATES PATENTS

|              |           |                |
|--------------|-----------|----------------|
| 2,114,161    | Antisell  | Apr. 12, 1938  |
| 2,482,308    | Wernlund  | Sept. 20, 1949 |
| 40 2,539,096 | Miller    | Jan. 23, 1951  |
| 2,654,146    | Mooradian | Oct. 6, 1953   |
| 2,697,130    | Korbelak  | Dec. 14, 1954  |
| 2,776,255    | Hammond   | Jan. 1, 1957   |
| 2,816,066    | Russell   | Dec. 10, 1957  |